

## UNITED STATES PATENT OFFICE.

CHARLES W. HEPPENSTALL, OF PITTSBURGH, PENNSYLVANIA, ASSIGNOR TO HEP-  
PENSTALL FORGE & KNIFE COMPANY, OF PITTSBURGH, PENNSYLVANIA, A COR-  
PORATION OF PENNSYLVANIA.

## ALLOY.

No Drawing.

Application filed March 7, 1925. Serial No. 13,857.

The particular object which I have in view is the provision of a new and improved alloy for use in operations involving the cutting, shaping or forming of hot steel, and which may be advantageously employed for such purposes in either cast or forged form. Thus my novel alloy is particularly adapted for making shear blades to be used for cutting hot steel, and for forming blocks for die-casting.

The alloy steels now employed for such purposes are usually alloys containing relatively high percentages of the more expensive alloy elements, such as tungsten, molybdenum, vanadium, &c.

My alloy is characterized by the use of relatively high amounts of the relatively inexpensive alloy elements, such as carbon and chrome in combination with hitherto-un-  
known small amounts of the more expensive elements, such as tungsten or molybdenum.

Thus I have discovered that the following analysis produces greatly improved results: carbon 1.50% to 2.25%, chrome 3.50% to 25 6%, tungsten 0.50% to 2%.

The elements manganese, silicon, phosphorus and sulphur, are employed within the limits commonly used in commercial alloy steels. These limitations are usually approximately as follows: manganese from .30% to 1.00%; silicon .01% to .50%; phosphorus from a trace to .06%, and sulphur from a trace to .06%.

Nickel may be present in amounts varying from a mere trace up to 1.50%. In many instances nickel is found in the steel scrap which is available today. This element causes only a very slight improvement in the performance of my new alloy, and I therefore classify it as a non-essential element, frequently present but not materially modifying the alloy. I prefer to keep the nickel below 0.25%.

The element molybdenum may be substituted for the tungsten, following the usual practice of using less of the former than of the latter, preferably about one-half. However, my experience has been that a better performance is obtained by using tungsten instead of molybdenum.

I have also found that a slight improvement in performance may be obtained by employing the element vanadium, but in my

judgment the added cost involved is not justified. If employed the vanadium is used in amounts from 0.10% to 0.50%.

My experience in the development of this high carbon-high-chrome alloy containing a small percentage of tungsten, through laboratory and plant experiment and tests, and through performance in service, has shown that it has exceptional ability to withstand service, such as the cutting or shearing of hot steel, the forming or shaping of hot metal of any kind, or in the casting of hot metal, as for example—any die casting work.

I term this alloy a "steel" because of the method of its manufacture and heat treatment, and the fact that in its physical properties, it exhibits the characteristics ordinarily attributed to steels; although its carbon content is above the range usually assigned to steels, and ordinarily it would be classed as cast iron, if it were judged only by its carbon content.

The uses to which the alloy has been put in service are those in which it has been customary, where the very best performance is demanded regardless of cost, to use expensive alloy combinations, particularly those high in tungsten. In the case of my novel alloy, which has shown better performance than any alloy heretofore used for the purpose, its unusual merit is due to the use of the large amounts of comparatively inexpensive elements such as carbon and chrome, and the very small amount of the expensive element tungsten or its equivalent in molybdenum.

The discovery of the fact that the beneficial effects of tungsten can be intensified by the use of large amounts of carbon and chrome, and that the resulting product has valuable properties resulting in performance superior to that of the most expensive alloy steels heretofore used, is the most striking feature of this invention.

Tests have demonstrated that this improvement is to the extent of from three hundred to four hundred per cent.

What I desire to claim is:—

1. An alloy for the purposes described comprising from 1.50% to 2.25% of carbon; from 3.50% to 6% of chrome, and from 0.50% to 2% of tungsten, and the principal part of the remainder being iron together

with manganese, silicon, phosphorus and remainder being iron together with manganese, silicon, phosphorus and sulphur <sup>10</sup> sulphur within the limits now employed in commercial steel.

2. An alloy for the purposes described comprising from 1.50% to 2.25% of carbon; from 3.50% to 6% of chrome; from 0.50% to 2% of tungsten, and from 0.10% to 0.50% of vanadium, and the principal part of the

within the limits now employed in commercial steel.

Signed at Pittsburgh, Pa., this 5th day of

March, 1925.

C. W. HEPPENSTALL.